

Patented Mar. 27, 1928.

1,664,034

# UNITED STATES PATENT OFFICE.

ARTHUR W. HUSEMAN AND THOMAS A. LEONARD, OF CHICAGO, ILLINOIS.

## PROCESS OF COATING MANUFACTURED PRODUCTS.

No Drawing.

Application filed June 19, 1922. Serial No. 569,429.

This invention relates to a new and improved process of coating manufactured products and has for its object to provide a new and improved process of this description. It often happens in practice that pieces of material, such for example as metal, must be covered with some suitable coating, and yet there are parts of the surface or surfaces upon which it is not desired to have this coating. One instance for example where such conditions prevail is where metal pieces are to be japanned or enameled and portions of such pieces are required to have no japan or enamel upon them, and in some instances these uncovered portions must be finished by a tool. It is the present practice to entirely cover the pieces of material with japan or enamel which is baked on it, and then put the pieces in the machine and finish these surfaces from which the coating has been removed. This process is expensive and requires the piece of material after being japanned or enameled to be put in the machine and handled, thus endangering the coating upon it. Again these pieces of material when going through the machining process, are handled a number of times and hauled around on trucks and are being put in and taken out of various machines and thrown on benches, all of which endangers the coating and makes it often necessary to recoat them.

One of the objects of the present invention is to provide a process by means of which the piece of material may be finished and have all the machine work done upon it before it is coated, and then coat it in such a manner that the portion of the coating on the parts which are to be free from the coating, can be easily and quickly removed.

The invention has other objects which are more particularly pointed out in the accompanying description and may be applied to any suitable material.

For purposes of illustration we will describe our invention in connection with japanning or enameling pieces of metal. When our invention is used these pieces of metal can first be completely finished. All the tool work required may be done upon it, and all plating of the parts may be done. When the piece of material is finished, the portion or portions thereof which are to be free from the coating when finished are covered with a gelatinous proteic substance, such for example as fish glue or the albu-

minoidal glue made from the hoofs, horns, feathers and hair of birds, or that made from the by-products in starch manufacture or any other suitable gelatinous proteic substance. All of the substances named are gelatinous proteic substances with coagulating properties, and are preferably used in liquid form and applied with a brush or in any suitable manner to that portion of the surface which it is desired to have free of the permanent coating. It is also desirable that this gelatinous proteic substance should have rapid drying qualities, and this may be secured by the addition of a small amount of alcohol thereto or any other substance which quickly evaporates. The surfaces which it is desired to have free of the permanent coating are covered with this gelatinous proteic substance. It is permitted to dry and then it is coated with shellac, enamel or other permanent coating desired. It is then baked, and the gelatinous substance forms a comparatively thick white bubbly mass which adheres to the surface of the piece of material, but which prevents the permanent coating from adhering thereto, and so acts upon the permanent coating as to make it easily removable by simply brushing with a brush or with the hand or with any suitable removing device.

After the baking the permanent coating at the point or points where the temporary coating is applied, is removed, as well as the temporary coating, leaving the material with a finished surface or surfaces at this point or these points. The removal of the coatings may be accomplished in any desired manner, as by a brush, rag or the like, or even by the hand, as they are in such condition that they can be easily rubbed off. If for example the piece of material has a hole with screw threads, this temporary coating will be applied to these screw threads, and then the entire piece may be dipped in or otherwise coated with the permanent coating material and then baked, and then the brush run through the hole, and this will quickly and easily remove both the permanent coating material and the temporary coating material, leaving the threads free and clean.

It will thus be seen that by means of this invention all handling of the material after the permanent coating is placed thereon is avoided and all the expense and danger to the injury thereof thus avoided. The

handling and finishing may all be completed, the final act being to put on the permanent coating.

It will further be noted that the area of surface to be left free of the permanent coating may be accurately determined, because this surface will depend upon the amount of the surface covered by the temporary coating, and when this portion of the surface is rubbed after baking, both coatings will quickly and easily come off, leaving a properly defined unbroken border line about the surface. In other words, the amount of coating to be rubbed off is determined by the area covered by the temporary coating and the additional border line of the permanent coating around this surface is also predetermined and may be made any shape desired and the party rubbing off the coatings need not be concerned as to the surface to be free, because such surface is determined entirely by the temporary coating and by the person who applies this temporary coating.

The invention is of great importance also in cases where portions of the surface must be plated with some material, such as nickel, silver or the like, as this plating may be accomplished before the permanent coating herein referred to is applied, the plated surface being covered with the temporary coating before the permanent coating is applied to the piece of material.

It will thus be seen that this invention may be applied to any suitable material where such material requires only partial coating whether due to the fact that it has some plated surface or surfaces, or some

surface or surfaces which must be machined, or some surface or surfaces which for any other reason must be free of the permanent coating herein referred to, and we have used the term "partial coating" as applying not to any plating or the like, but to the final permanent coating put on over the entire surface; including that to which the temporary coating is applied, but which when the product is finished covers only a part of the device due to the fact that the portion thereof over the temporary coating has been removed.

We claim:

The process of coating metal, parts of which must be machined, so that the portion of the coating from the machined parts may be easily removed, which consists in first machining the parts to be machined and then applying a coating of gelatinous, proteic substance in a liquid form to the portions of the surface of the metal that have been machined from which the permanent coating is to be removed; then coating with the permanent enamel in a liquid form the entire surface to be coated, including the machined surface on which the gelatinous, proteic substance is placed, then heating the metal and coating, until the gelatinous, proteic substance forms a white, bubbly mass thicker than the enamel coating at the points free from the gelatinous, proteic substance, and then brushing the bubbly mass from the surface of the metal so as to leave it exposed.

ARTHUR W. HUSEMAN.  
THOMAS A. LEONARD.